

# UNITED STATES PATENT OFFICE.

EUGÈNE SCHNEIDER, OF LE CREUZOT, FRANCE.

## GAS-CHECK PAD FOR GUN BREECH-BLOCKS AND PROCESS OF MAKING SAME.

1,229,662.

Specification of Letters Patent. Patented June 12, 1917.

No Drawing.

Application filed December 9, 1916. Serial No. 136,119.

To all whom it may concern:

Be it known that I, EUGÈNE SCHNEIDER, a citizen of the Republic of France, residing at Le Creuzot, France, have invented a new 5 and useful Improvement in Gas-Check Pads for Gun Breech-Blocks and Processes of Making Same, which is fully set forth in the following specification.

The pad that constitutes the plastic element of the well-known de Bange gas check is generally composed of a core formed of a mixture of asbestos and tallow inclosed in a casing of fabric or cloth.

The check ring pads of that kind have 5 considerable drawbacks: their volume increases under the influence of heat, the expansion being often such as to produce rapidly an inconvenience in the working of the breech blocks, while on the other hand, after 0 a prolonged period of firing, they lose a part of their tallow, with the result that the jointing becomes defective and the casings are cut and burn.

It has been attempted to remedy those 5 drawbacks by employing in place of the tallow, a grease produced by saponifying colza oil with soda. This greasy substance, when mixed with the asbestos, has the drawback of being soluble in water, which circumstance renders the preservation of the pads very difficult, especially when the casings are not quite tight.

Now according to the present invention the gas check pads are made of a peculiar 5 substance which, while being as plastic as the usual materials hitherto employed, has not the drawback of swelling or hardening during the firing nor of deteriorating rapidly under the action of moisture.

0 This new substance consists of asbestos impregnated with a soap that is insoluble in water, such as for instance a lime soap mixed with vaseline or equivalent fatty substance, the impregnation of the asbestos with the 5 insoluble soap being facilitated by dissolving the soap in ether or any other suitable solvent.

The insoluble soap is preferably a lime soap, but it may also be a soap having as its 0 basis baryta, magnesia, or a metal such as lead, zinc, etc.

The soap is prepared by saponifying 5 wholly or partially a natural fatty substance (such as oil, grease, or wax) by the corresponding metallic oxid, or by double decomposition between an aqueous solution

of ordinary soap (soda soap or potash soap) and a soluble salt of the selected metal. The resulting soap may then be mixed with a determined excess of a fatty substance. 60

This fatty substance is preferably vaseline; but the latter may be replaced wholly or partly by heavy oils of petroleum, shale or coal tar, or by paraffin, ceresin, etc., or by a mixture of these substances. 65

The following is a description of the preferred process of preparation and the constitution of the improved gas check pads.

The pads formed of a mixture of lime soap and vaseline are made as follows: 70

A lime soap is made by pouring into a vessel ordinary colza oil and about 13% of powdered slaked lime.

This mixture is heated for about two hours, being frequently agitated for the purpose of facilitating saponification, and the temperature of the heating being sufficiently high to insure that the mixture shall remain sufficiently fluid during the whole of the operation. When it is considered that the saponification is complete, the impurities and more particularly any uncombined lime, is removed by skimming. 80

The percentage of lime in the resulting soap should be about 8%. It may be determined by titration. If the percentage is too great, the requisite quantity of colza oil is added, when the whole is melted again with stirring. 85

The lime soap of the desired percentage, 90 after being suitably cooled, is dissolved in a suitable solvent in order that the asbestos fibers shall become completely impregnated with the soap. It is preferred to use ether as the solvent, in the proportion of about one 95 and a half liters to one kilogram of plastic material to be made. Other solvents, such as petroleum ether or petroleum spirit or petrol, or even benzin may be used.

The solution is passed through a metal 100 cloth for the purpose of separating out the insoluble portions.

To this solution there is added asbestos in quantity four times the weight of that of the lime soap. The asbestos and the soap solution are mixed very intimately together, and then the ether is evaporated without exceeding a temperature of 60° C. 105

The block of material thus formed is crumbled, for instance by rubbing it on cotton carding cards; then the crumbled mixture is mixed with vaseline. 110

The vaseline may also be incorporated at the same time as the soap, by dissolving the two substances together in ether and then adding the asbestos. The ether is finally driven off by evaporation.

In order that the mixture shall be perfectly homogeneous, the process is carried out bit by bit. Alternate layers of the material and vaseline are applied one on top of 10 the other, and the mixture is intimately kneaded together after each addition of material and vaseline.

The process of making a gas check pad for gun breech blocks from the plastic material hereinbefore described, may be as follows:—

A strip of annealed metal cloth is cut and fluted on the proper sides, and placed in the finishing die.

The pad, preferably roughly shaped at its 20 edges, is placed in the die, the flutes are pressed down and finally "nailed" down. The pad is then subjected to the final compression.

Having now described my invention, what 25 I claim as new and desire to secure by Letters Patent is:—

1. A gas check pad for guns comprising asbestos, water-insoluble soap incorporated therewith and a fatty substance to impart 30 plasticity thereto.

2. A gas check pad for guns comprising asbestos, lime-soap and a fatty substance to impart plasticity thereto.

3. A gas check pad for guns comprising asbestos, lime-soap and vaseline to impart 35 plasticity thereto.

4. A gas check pad for guns comprising 80 parts of asbestos, 20 parts of colza-oil lime-soap containing about 8 per cent. of lime and a fatty substance to impart plasticity thereto.

5. The process of making gas check pads for guns consisting in impregnating asbestos with a water-insoluble soap dissolved in a volatile solvent, evaporating off the solvent and then incorporating the product in successive small portions into vaseline to render the mass plastic.

6. The process of making gas check pads for guns consisting in impregnating asbestos with a water-insoluble soap dissolved in a volatile solvent, evaporating off the solvent and then incorporating the product in successive small portions into a fatty body to render the mass plastic.

7. The process of making gas check pads for guns consisting in impregnating asbestos with a water-insoluble soap and vaseline dissolved in a volatile solvent and then evaporating the solvent.

8. The process of making gas check pads for guns consisting in impregnating asbestos with colza-oil lime-soap dissolved in ether, evaporating off the ether and mixing the product with vaseline to render the pad plastic.

9. The process of making gas check pads consisting in incorporating asbestos with colza-oil lime-soap prepared by heating colza-oil with about 13% of its weight of slaked lime, combining the excess of lime with additional colza-oil to reduce the lime in the soap to about 8% and then mixing the product with vaseline to render the pad plastic.

In testimony whereof I have signed this specification in the presence of two subscribing witnesses.

EUGÈNE SCHNEIDER.

Witnesses:

CHAS. P. PRESSLEY,  
ANDRÉ MOSTICKER.